

R. L. WHITEHEAD,  
ELECTROLYTIC REFINING OF TIN,  
APPLICATION FILED MAY 4, 1915.

1,157,830.

Patented Oct. 26, 1915.

2 SHEETS—SHEET 1.

*Fig. 1.*



*Inventor.*

Robert L. Whitehead  
By *James Davis & Marvin*  
*Attnys.*

R. L. WHITEHEAD.  
ELECTROLYTIC REFINING OF TIN.  
APPLICATION FILED MAY 4, 1915.

1,157,830.

Patented Oct. 26, 1915.

2 SHEETS—SHEET 2.



Fig. 2.



Inventor:  
Robert L. Whitehead  
By *James Davis & Marvin*  
*Attnys.*

# UNITED STATES PATENT OFFICE.

ROBERT L. WHITEHEAD, OF PERTH AMBOY, NEW JERSEY, ASSIGNOR TO AMERICAN SMELTING & REFINING COMPANY, OF MAURER, NEW JERSEY, A CORPORATION OF NEW JERSEY.

## ELECTROLYTIC REFINING OF TIN.

1,157,830.

Specification of Letters Patent.

Patented Oct. 26, 1915.

Application filed May 4, 1915. Serial No. 25,671.

To all whom it may concern:

Be it known that I, ROBERT L. WHITEHEAD, a citizen of the United States, residing at Perth Amboy, county of Middlesex, State of New Jersey, have invented certain new and useful Improvements in Electrolytic Refining of Tin; and I do hereby declare the following to be a full, clear, and exact description of the invention, such as will enable others skilled in the art to which it appertains to make and use the same.

My invention relates to certain new and useful improvements in the production of electrolytically refined tin from impure tin cast in the form of anodes.

In the practice of the invention, I first produce from the impure tin itself, an electrolyte of such a character that it will insure the continued maintenance of the electrolytic deposition of the tin during the refining operation and which will itself be devoid of lead, which is an impurity usually present in the tin to be refined. So also, after the electrolyte has been initially produced, I maintain its purity, during the refining operation, by still further continuing to exclude the entrance of lead from the tin anodes into the electrolyte. The tin anodes usually contain gold, silver, or other values, in addition to lead, and I find that all of these adhere for the most part, as slimes, to the anodes, and may be removed therewith at the termination of the electrolytic treatment; or, in part, they fall to the bottom of the electrolytic tank, from which they may be withdrawn, when occasion requires.

The expedient that I employ for preventing the entry of lead into solution in the electrolyte from the impure tin anodes is to employ in the electrolyte, during its preliminary formation and subsequently during the deposition of the tin therefrom upon the cathodes an agent which will convert the lead into a compound insoluble in the electrolyte. The agent that I prefer to employ for the purpose is sulfuric acid, which serves to convert the lead into lead sulfate, insoluble in the electrolyte which I employ, as will hereinafter more fully appear.

In the accompanying drawings, I have illustrated a form of apparatus suitable for the practice of the invention.

Figure 1 represents a top plan view of the

apparatus; Fig. 2 represents a sectional view of said apparatus on a plane indicated by the line 2—2 of Fig. 1; and Fig. 3 represents a sectional view on the plane indicated by the line 3—3 of Fig. 1.

Similar letters of reference indicate similar parts throughout the several views.

Referring to the drawings, it will be noted that they show, for convenience of illustration, a plurality of electrolytic vats or receptacles A arranged alongside of each other and provided with a protective lining a of mastic or other material neutral to the electrolyte. Within these receptacles are located the series of impure tin anodes b alternating with a corresponding series of cathodes c,—d indicating the location of the bus-bar with which the primary series of the anodes makes connection.

I employ as the electrolyte, a solution obtained by dissolving metallic tin in hydrofluosilicic acid. To obtain this electrolyte, I may conveniently make use of the apparatus shown in the drawings, wherein the anodes b are of the impure tin to be refined, and wherein the cathodes c are contained within cells e of porous earthenware or the like supported from the bottom of the vat upon glass insulator blocks f. To maintain the porous cells in position upon the glass insulator blocks it will be convenient, as shown, to provide the cathode bars g with clips h of sheet metal which prevent the cups from shifting their position. So also, clips i serve to support the cathode sheets from the cathode bars.

In preparing the electrolyte from the impure tin anodes, I may employ cathodes either of tin, copper, lead, or other appropriate metal. In the main body portion of the vats A and also in the porous cells e, I employ a 20% solution of hydrofluosilicic acid, containing .1% by weight of sulfuric acid. An electric current of suitable voltage and amperage is then applied until, upon testing, the solution has taken up 6% by weight of tin whereupon the passage of the current is then discontinued. During this preliminary formation of the electrolyte, the sulfuric acid contained in the solution combines with the lead which would otherwise go into solution in the electrolyte and converts it into lead sulfate which is insoluble

therein. The electrolyte thus produced consists of tin dissolved in hydrofluosilicic acid, and has been formed from the impure tin anodes without bringing any of the lead into solution. The electrolyte is therefore adapted to deposit pure tin upon cathodes, provided that it is further protected during the depositing operation from contamination by lead.

10 After the formation of the electrolyte, the porous cells *c* are removed, and cathodes, preferably of tin are suspended freely in the electrolytic vats to receive the deposition of the tin. The removal of the porous cells 15 permits the lowering of the voltage of the current to one-half a volt in lieu of the four to five volts employed during the formation of the electrolyte. The electric depositing current being then applied to the apparatus, 20 the tin in a pure state is deposited upon the cathodes from the impure anodes, and the purity of the electrolyte is insured by maintaining in solution therein a quantity of sulfuric acid appropriate to the conversion of 25 the lead of the progressively dissolving anodes into lead sulfate. As hereinbefore noted, the lead sulfate and the other values contained in the anodes adhere for the most part to the anodes, as slimes,—very little, if 30 any, of these constituents falling off into the vats. This is a feature of importance in the operation for the reason that at the termination of the operation, these slimes can be raised out of the solution because of their 35 adhesion to the practically exhausted anodes, so that the annoying inconvenience of removing slime deposits from the bottom of the vats is correspondingly decreased.

What I claim is:

40 1. In the electrolytic refining of impure tin containing lead, the method of producing an appropriate electrolyte for the refining operation, which consists in passing an electric current of suitable voltage and amperage from the impure tin as an anode to a cathode through an electrolyte which is a solvent of tin and lead, and protecting the electrolyte from contamination by lead, by incorporating with the electrolyte an agent 45 which will combine with the lead to form an insoluble compound; substantially as described.

50 2. In the electrolytic refining of impure tin containing lead, the method of producing an appropriate electrolyte for the refining operation, which consists in passing an electrolytic current of suitable voltage and amperage from the impure tin as an anode to a cathode through a solution of hydrofluosilicic acid containing an agent which will combine with the lead to form an 55 insoluble compound; substantially as described.

60 3. In the electrolytic refining of impure tin containing lead, the method of produc-

ing an appropriate electrolyte for the refining operation, which consists in passing an electrolytic current of suitable voltage and amperage from the impure tin as an anode to a cathode through a solution of hydrofluosilicic acid containing an amount of sulfuric acid sufficient to combine with the lead to form lead sulfate; substantially as described.

65 4. In the electrolytic refining of impure tin, the method of preventing contamination of the tin deposited from the impure tin anode upon the cathode, which consists in employing an electrolyte which is a solvent of tin and lead, and incorporating in 70 the electrolyte a protective agent sufficient to convert the lead contained in the dissolving tin anode into a compound insoluble in the electrolyte; substantially as described.

75 5. In the electrolytic refining of impure tin, the method of preventing contamination of the tin deposited from the impure tin anode upon the cathode, which consists in employing as the electrolyte a solution of 80 tin in hydrofluosilicic acid together with a protective agent sufficient to convert the lead contained in the dissolving tin anode into a compound insoluble in the electrolyte; substantially as described.

85 6. In the electrolytic refining of impure tin, the method of preventing contamination of the tin deposited from the impure tin anode upon the cathode, which consists in employing as the electrolyte a solution of 90 tin in hydrofluosilicic acid together with a quantity of sulfuric acid sufficient to convert the lead of the dissolving anode into lead sulfate; substantially as described.

95 7. The process of producing an appropriate electrolyte for the refining of impure tin, which comprises passing an electrolytic current of suitable voltage and amperage from a tin anode to a cathode through a solvent 100 adapted to take the tin into solution on passage of the current, and interposing a porous diaphragm between the anode and cathode during the process; substantially as described.

105 8. The process of producing an appropriate electrolyte for the refining of impure tin, which comprises passing an electrolytic current of suitable voltage and amperage from a tin anode to a cathode through a solution of hydrofluosilicic acid, and interposing a porous diaphragm between the anode and cathode during the process.

110 9. An electrolyte for the deposition of tin free from lead, comprising an electrolytic solution of tin in hydrofluosilicic acid containing an agent which will combine with lead to form an insoluble compound; whereby, upon the passage of a current there-through from an impure tin anode containing lead to a cathode, the tin will be dis-

solved from the anode and deposited on the cathode without contamination with lead; substantially as described.

10. An electrolyte for the deposition of tin free from lead, comprising an electrolytic solution of tin in hydrofluosilicic acid containing a small amount of sulfuric acid; whereby, upon the passage of a current

therethrough from an impure tin anode containing lead to a cathode, the tin will be dissolved from the anode and deposited on the cathode without contamination with lead; substantially as described.

In testimony whereof I affix my signature.

ROBERT L. WHITEHEAD.